

A. R. HUNT & J. H. GROSE,  
METHOD OF FORGING WHEELS,  
APPLICATION FILED AUG. 1, 1911.

1,140,681.

Patented May 25, 1915.



Witnesses:

Geo. C. Davies

M. P. Alexander

Inventors

A. R. Hunt

J. H. Grose

By Lathicium, Bett & Fuller

576595

# UNITED STATES PATENT OFFICE.

AZOR R. HUNT AND JAMES H. GROSE, OF MUNHALL, PENNSYLVANIA.

## METHOD OF FORGING WHEELS.

1,140,681.

Specification of Letters Patent.

Patented May 25, 1915.

Application filed August 1, 1911. Serial No. 641,782.

To all whom it may concern:

Be it known that we, AZOR R. HUNT and JAMES H. GROSE, both citizens of the United States, and residing at Munhall, in the county of Allegheny and State of Pennsylvania, have invented certain new and useful Improvements in Methods of Forging Wheels, of which the following is a specification.

10 Our invention relates to the manufacture of forged metal wheels and more particularly of flanged metal car wheels. Heretofore, in forging such wheels, the blanks from which the wheels are made have according 15 to some methods been compressed and shaped by simultaneously working or displacing the metal from both sides inwardly, or, in other words, both sides of the wheels have been shaped at the same time. In forging 20 wheels in this manner, the metal flows unevenly and owing to the lack of control in the flow, the metal is frequently so irregularly disposed in expanding or increasing its diameter during the shaping operations as 25 to "overfill" and form a fin or series of fins on one side of the axial center of the blank with a corresponding "underfilling" or lack of material at other points on the periphery of the partly formed blanks. The formation 30 of such fins on the blanks results in making defective wheels and is the cause of considerable expense in the manufacture of such wheels. The irregular flow of the metal also frequently permits the axially central 35 portion of the blanks, in which the segregated portions and poorest quality of the metal is located, to be displaced sidewise to such extent as to eventually be located in the web portion of the finished wheel, another 40 very undesirable feature.

One object of our invention is to provide a method of forging wheels having a novel series of steps whereby the flow of the metal in the blanks is regulated and controlled to 45 a much greater extent than has been heretofore found possible and by the use of which the blanks are compressed uniformly to a practically constant or uniform thickness and the formation of defective wheels there- 50 by very largely overcome and prevented.

In forging wheels by our improved method, the blank which may be cylindrical or polygonal in cross section and of any desired diameter and thickness, is first reduced 55 in thickness and by this first forging step one side only of the blank is shaped or

changed in contour. The so formed and partly shaped blank is then transferred to another set of dies where the web and tread are partly formed. After the first forging 60 operation by means of which a rudimentary hub is formed on one face, the metal forming the central portion of the blank remains undisturbed, that is the thickness of the blank at its center portion after the first 65 forging operation is substantially the thickness of the hub in a finished wheel. It will be noted that because of this many advantages are gained; first the metal in the center of the blank which metal contains the 70 segregated metalloids, pipes or irregularities, forms the final hub of the wheel where the mass of metal is present and is not forced into the web, tread or flange; second, in the punching of the blank for the purpose 75 of providing the axle opening much of the inferior metal is removed, and, third, it will be seen that the forging action is in the natural lines, that is the flow of the metal is all downward and away from the center 80 or hub. In following this method it has been found that there is absolute uniformity in the product, all portions of the die being completely filled.

In order that our invention may be more 85 readily understood, we have shown in the accompanying drawings illustrations of the steps herein described and claimed, in which,

Figure 1 is a diagrammatic sectional view of a pair of forging dies having an un- 90 formed blank seated therein. Fig. 2 is a similar view showing the second step, in which the metal in the blank has been displaced and fits the female die. Fig. 3 is a view showing the next step wherein the 95 partly formed blank has been placed in a die of larger diameter; Fig. 4 shows the completion of the steps as contemplated by this method; Fig. 5 is a view of a blank such as contemplated by us; Fig. 6 is a view of 100 the blank in the form in which it is removed from the die of Fig. 2, and, Fig. 7 is a view of the partly finished wheel in the form in which it is removed from the dies of Fig. 4.

In carrying out our method we prefer to 105 employ any well known forging devices. In the first machine we provide an upper die 10 having a flat forging face 11. The lower die 12 is of comparatively small diameter with relation to the diameter of a finished 110 wheel and contains a concentric recess 13 within which the metal forming the hub of

the wheel is forced. Within the die 12 is shown an unformed blank 14.

Referring to Fig. 2 it will be seen that the die 10 has caused the metal of the blank 14 to flow evenly through all the spaces within the lower part of the die opening thus leaving the partly formed blank 15 with a rudimentary hub 16 and the outlines of the face of the wheel formed on one side thereof. The upper face 17 is substantially a plane surface.

Referring to Fig. 3 it will be seen that a new set of dies has been substituted. The upper die 18 is provided with a concentric projection 19 which is adapted to contact the plane surface 17 of the blank and outline the remainder of the hub. The opening in the lower die 20 is of greater diameter than the opening in the die 12. This die has a concentric projection 21 corresponding to the projection 19 on the die 18. The sides 22 of the die opening are flared and, at 23, provision is made for the forming of a rudimentary flange.

In Fig. 4 the dies 18 and 20 have caused the metal in the blank 15 to fill the die opening, the forging action as will be seen being downward and away from the common center of the dies and the blank. It will be seen that a partly formed wheel 24 is produced and that the metal forming the hub has not been disturbed from the center of the wheel. The hub of the partly finished wheel is of the same thickness as the metal at the center of the blank as formed by the dies of Fig. 2. It will be understood that the partly formed wheel 24 is afterward further operated upon to produce a finished product but as such steps do not concern the present invention we shall not describe nor illustrate the same.

The advantages of our invention arise from the manner of displacing the metal uniformly in forming the hub and web portions of the wheel at the beginning of the wheel forging operations. By first shaping one face of the blank to the contour desired for the hub and web portions of the wheel,

and then, in a second or later forging step, forming the opposite face of the blank to the desired contour for the hub and web portion of the wheel, the metal is caused to flow downwardly and away from the axial center of the blank and be distributed equally about the axis of the blank and wheel, and blanks of uniform thickness are provided.

By employing the forging steps as described by our invention the blanks are finished in the subsequent forging steps to a uniform diameter and thickness and "overfilling" or "underfilling" caused by unequal sidewise flow of the metal is overcome and prevented, while the metal in the axial center of the unformed blanks remains in the same relative location in the forged wheel or is removed in the operation of punching the hub to form the axle eye of the wheel.

Modifications in the form and arrangement of the forging dies and in the number of forging steps employed may be made without departing from our invention as defined in the claim.

We claim:

In the manufacture of forged wheels the steps consisting in subjecting a cylindrical blank having substantially flat plane end surfaces to a series of successive forging steps to lessen the thickness and increase the diameter of the blank, shaping one end surface of the blank without shaping the opposite end surface in the first of the series of steps, and then further reducing the thickness and increasing the diameter and shaping the opposite end surface of the blank in a later step and then subjecting the blank to further forging steps in shaping the rim or periphery of the blank to size and contour.

In testimony whereof, we have hereunto set our hands.

AZOR R. HUNT.  
JAMES H. GROSE.

Witnesses:

A. A. COREY, Jr.,  
W. J. HULL.